

## 1

3,194,655

## PROCESS FOR MAKING A COPPER-CHROMIUM-ZIRCONIUM ALLOY

Alan R. Pels, Stamford, and Herman F. Petsch, New-town, Conn., assignors to National Distillers and Chemical Corporation, Richmond, Va., a corporation of Virginia

No Drawing. Filed July 28, 1961, Ser. No. 127,477

3 Claims. (Cl. 75—135)

This invention relates to copper-chromium-zirconium alloys.

The object is to provide such an alloy with its components proportioned to provide the maximum possible degree of high electrical conductivity, resistance to undue softening when working at high service temperatures, such as in the vicinity of 400° C., and high notch strength or toughness.

The above properties are desirable when the alloy is used to make commutator segments for electric motor armatures which must operate at high rotative speeds and high temperatures. They are also desirable when the alloy is used for brazing or welding in the case of work which in service must conduct electricity while mechanically stressed under high temperatures. The desirable properties of the new alloy make its use advisable whenever these properties are an advantage.

The prior art has suggested in general terms the addition of zirconium to copper-chromium alloys. However, this has been insufficient to teach the art enough to permit the production of an alloy suitable for commercialization. Commercially there are only the copper-zirconium and copper-chromium alloys available for use as electric conductors operating under high stress at elevated temperatures and comparable service. The former is lacking in strength, while the copper-chromium alloy lacks notch toughness and resistance to undue softening at high temperatures.

According to the present invention the object stated hereinabove is attained by an alloy consisting, by weight, of from .60 to .90% pure chromium, .40 to .60% pure zirconium and with the balance pure copper. Insofar as is commercially possible, the alloy is free from oxygen in any form. For use it is solution heat treated and quenched, and then ordinarily it is cold worked and aged. Such processing may be varied. The components are pure to the degree that this is now commercially possible, and the alloy is free from other components excepting possible traces.

Within the above compositional ranges, it follows that the chromium content cannot be less than the zirconium content. Furthermore, the zirconium must be present in metallic form as contrasted to zirconia resulting from the use of zirconium for the purpose of de-oxidizing a copper-chromium alloy. The best possible results are believed to be obtained with an alloy consisting of .75% pure chromium and .50% pure zirconium, the balance of course being pure copper and the alloy being oxygen free.

To make certain that the zirconium is present in its metallic form, any oxygen present in the copper prior to the addition of this alloying component should be removed by de-oxidation. Casting of the melt should be done so as to avoid an oxygen pick-up.

The new alloy has been made in the following manner:

The copper may be cathodic copper, OFHC copper or

## 2

tough pitch copper, all of which are substantially pure. The copper is melted down while protected from oxygen, as by being kept under a cover of charcoal floating on its surface. Its temperature is brought to about 1100° C. and it is then de-oxidized by adding small amounts of any suitable commercial de-oxidizer that would ordinarily be used to scavenge oxygen from copper. A calcium-lithium type is suitable. The temperature is then raised to about 1500° C., when the copper is again de-oxidized. Throughout this procedure good metallurgical techniques are used to obtain an oxygen free copper that is free from everything except possibly traces of the de-oxidizer or de-oxidizers used.

With the copper at about 1500° C., the selected amount of chromium is added. This may be in the form of pure chromium powder wrapped in pure copper foil. Commercial copper-chromium master alloy may also be used, containing from 5 to 10% chromium with the balance copper. This addition is made through the charcoal cover. The melt is held at about 1500° C. long enough to make certain that the chromium is completely dissolved in the copper, this high temperature having the advantage of reducing the solution time.

Next the melt is permitted to cool to about 1300° C., this temperature being high enough to provide rapid solution of the zirconium and is of value in reducing the zirconium loss due to possible small amounts of oxygen which may be present in the melt in spite of the precautions used to avoid this. The selected amount of pure zirconium is added at this time. This may be in the form of copper-zirconium master alloy containing about 33% zirconium with the balance copper. Again for the purpose of making as certain as possible that zirconium loss is avoided, the melt is poured just as soon as the zirconium goes completely into solution. It is possible to top pour the melt while holding the charcoal cover back.

It is believed to be preferable to protect the melt against oxygen while pouring. However, it has been found that if the pouring time is short, and the pouring stream is kept solid, as contrasted to spraying, such protection is not mandatory. The cast metal may be permitted to solidify without requiring any particular protection from oxygen since the top surface exposed to the atmosphere is ordinarily of relatively small area. In any event, any oxygen picked up by the top of the casting is localized and does not affect the balance of the casting.

After solidification the casting is extruded at temperatures of about 930° C. This temperature is used not only to permit extrusion without using excessive extrusion force, but also because it assures keeping the chromium and zirconium in complete solution with the copper. Instead of extrusion, hot rolling or forging is also possible. After such working the alloy is air cooled.

In the actual working of the present invention the casting is extruded to a rectangular shape that is 2" wide and .50" thick. It is air cooled after extrusion largely as a matter of convenience. Thereafter it is solution heat treated by being heated to about 950° C. for about 1½ hours. The shape is actually in the necessary furnace somewhat longer, the 1½ hours time period being while the metal is actually at 950° C. At the end of the described time period the metal is quenched in water to keep the chromium and zirconium in solution with the copper. If the cooling is too slow there is a risk that the alloying components might come out of solution.

The extruded shape is then cold rolled to .25" thickness, its 2" width remaining the same. It is thereafter given a treatment corresponding to that already described and after that the shape is further cold rolled to .100" thick, its width again remaining at 2". Then to make absolutely certain that the chromium and zirconium are in solution, the .100" thick material is solution heat treated again as described above but in this instance using a time of 3 hours at the 950° C. temperature. Possibly this prolonged solution heat treatment is unnecessary but it has been considered to be a wise precaution. Here again the work is water quenched from its heat treatment temperature to hold the alloying components in solution.

The .100" thick material is next cold rolled to give varying tempers. It has been rolled to thicknesses of .090, .070, .040 and .020 of an inch. Following such cold rolling the material is aged by heating it to 1 hour, at temperatures ranging from 450° C. to 600° C.

A specific example of the results achieved is as follows:

The specimen had a composition of .60% chromium, .45% zirconium and the balance copper. The chromium and zirconium were present in pure metallic form and the alloy contained no appreciable or easily measurable amount of oxygen in any form. It was substantially free from anything other than specified, with the understanding that the balance was, of course, pure copper. In this instance the material was rolled to the .04" thickness from which 1/2" wide specimens were cut.

These specimens were given varying ageing heat treatments so that they broke down into the following categories:

A—As cold rolled only

B—As cold rolled only and aged for 1 hour at 450° C.

C—As cold rolled only and aged for 1 hour at 600° C.

These three specimens showed the following conductivities:

A=35.5

B=73.6

C=81.2

The above are in percent I.A.C.S. at 20° C.

It can ordinarily be assumed that hardness at room temperature after an ageing high temperature treatment means lack of softness at high service temperatures because otherwise recrystallization would occur during the ageing treatment and result in softness at both room and high temperatures. With this in mind the following hardness values were obtained:

A—Rockwell B 82.0

B—Rockwell B 84.0

C—Rockwell B 76.0

Tensile testing at room temperature produce the following values:

A—61,700 p.s.i.

B—76,000 p.s.i.

C—61,350 p.s.i.

Elevated temperature tensile testing of the B specimen showed at 450° C. a tensile strength of 53,500 p.s.i.

In addition to the above, one of the B specimens was cut to a .700" width and had 60 degree V-notches formed in its edges reducing its width at the roots of the two notches to .500". This notched B specimen when tested at 450° C. showed a tensile strength of 56,600 p.s.i.

Two C specimens were also tensile tested at 450° C., one being unnotched and the other notched as just described in the case of the B specimen. In this instance the unnotched specimen showed a tensile strength of 40,900 p.s.i. and the notched specimen showed 45,250 p.s.i.

It can be appreciated from the foregoing that the object of the invention is achieved by the compositional balance described in conjunction with the use of good practices assuring that the resulting alloy is free from

oxygen and other than mere traces of de-oxidizers and the like which are unavoidable.

It is necessary to keep the composition within the ranges specified. If the chromium is permitted to drop below the .60% minimum the mechanical properties reduce without a proportionate gain in electrical conductivity. Chromium above .90% causes an excessive loss in electrical conductivity without a proportionate gain in mechanical properties. If the zirconium drops below the .40% minimum or goes above .60% the resistance to high temperatures suffers.

Finally, if the chromium content is reduced to less than the zirconium content, then at high temperatures, such as around 400° C. or higher, the tensile properties drop to a substantial degree thus indicating undue softness when the alloy is in service at such high temperatures.

Although the alloying, heat treatment, and other processing have been described in some detail, it is believed possible to vary these somewhat. It is necessary, neglecting traces of de-oxidizers, etc., to obtain an alloy consisting only of from .60 to .90% chromium, .40 to .60% zirconium, balance copper. Oxygen is avoided as much as possible keeping in mind that the zirconium in particular has a great tendency to combine with oxygen. The new alloy requires that the zirconium, and the chromium also, be in metallic form and thoroughly in solution with the copper. If these precautions are observed, it is believed that the new alloy may be handled generally in the manner of the old copper-chromium and copper-zirconium alloys, with the resulting new material avoiding the disadvantages of both of these old alloys. Ordinarily, the new material will be solution heat treated, to assure the condition of complete solution of its components, and it would ordinarily be cold worked to temper it somewhat and then, by the use of heat and time, aged to enhance its physical and electrical properties to the optimum degree.

We claim:

1. A process for making a copper-chromium-zirconium alloy, comprising forming a melt of substantially pure oxygen free copper protected from oxygen, while maintaining said melt so protected and at a high temperature completely dissolving therein from .60 to .90% chromium, thereafter while so protected lowering the temperature of said melt to a temperature causing rapid solution of zirconium therewith without excessive zirconium loss and dissolving therein from .40% to .60% zirconium and with complete solution thereof promptly processing the alloy melt to form a casting.

2. A process for making a copper-chromium-zirconium alloy, comprising forming a melt of substantially pure oxygen free copper protected from oxygen, while maintaining said melt so protected and at a high temperature completely dissolving therein from .60 to .90% chromium, thereafter while so protected lowering the temperature of said melt to a temperature causing rapid solution of zirconium therewith without excessive zirconium loss and dissolving therein from .40% to .60% zirconium and with complete solution thereof promptly processing the alloy melt to form a casting, and thereafter reducing said casting to the shape and dimensions desired and solution heat treating this shape.

3. A process for making a copper-chromium-zirconium alloy, comprising forming a melt of substantially pure oxygen free copper protected from oxygen, while maintaining said melt so protected and at a high temperature completely dissolving therein from .60 to .90% chromium, thereafter while so protected lowering the temperature of said melt to a temperature causing rapid solution of zirconium therewith without excessive zirconium loss and dissolving therein from .40% to .60% zirconium and with complete solution thereof promptly processing the alloy melt to form a casting, and thereafter reducing said casting to the shape and dimensions desired and solution heat treating this shape.

65 4. A process for making a copper-chromium-zirconium alloy, comprising forming a melt of substantially pure oxygen free copper protected from oxygen, while maintaining said melt so protected and at a high temperature completely dissolving therein from .60 to .90% chromium, thereafter while so protected lowering the temperature of said melt to a temperature causing rapid solution of zirconium therewith without excessive zirconium loss and dissolving therein from .40% to .60% zirconium and with complete solution thereof promptly processing the alloy melt to form a casting, and thereafter reducing said casting to the shape and dimensions desired and solution heat

treating this shape and thereafter cold working and aging the shape.

References Cited by the Examiner

UNITED STATES PATENTS

|           |       |               |        |
|-----------|-------|---------------|--------|
| 724,524   | 4/03  | Tilden        | 75-135 |
| 2,025,662 | 12/35 | Hensel et al. | 75-153 |
| 2,066,512 | 1/37  | Archer        | 75-153 |
| 2,254,944 | 9/41  | Hensel et al. | 75-153 |

OTHER REFERENCES

Dennis, "Metallurgy of the Non-Ferrous Metals," Sir Isaac Pitman & Sons, Ltd., London, 1953, pp. 154-155.

5 DAVID L. RECK, *Primary Examiner.*

RAY K. WINDHAM, ROGER L. CAMPBELL,  
*Examiners.*